

[54] CRUDE OIL HEAT EXCHANGE

[75] Inventor: Russell F. Stedman, Des Plaines, Ill.

[73] Assignee: Universal Oil Products Company,  
Des Plaines, Ill.

[22] Filed: Jan. 24, 1972

[21] Appl. No.: 220,455

[52] U.S. Cl..... 208/47, 165/1, 165/134,  
203/7, 208/48 AA, 208/348

[51] Int. Cl..... C10g 9/12, C10g 9/16

[58] Field of Search..... 208/47; 203/7;  
165/95, 1, 134

## [56] References Cited

## UNITED STATES PATENTS

|           |        |                |          |
|-----------|--------|----------------|----------|
| 2,938,851 | 5/1960 | Stedman et al. | 208/47   |
| 2,499,435 | 3/1950 | Whitacre       | 208/47   |
| 3,024,171 | 3/1962 | Bone           | 208/47 X |
| 2,414,761 | 1/1947 | Nutting et al. | 203/7    |

|           |         |          |          |
|-----------|---------|----------|----------|
| 2,534,905 | 12/1950 | Friedman | 203/7 X  |
| 2,947,686 | 8/1960  | Phillips | 203/7 UX |

## OTHER PUBLICATIONS

Parker, Ivy M., National Petroleum News, "Refinery Corrosion Problems Reviewed," Sec. 2, June 7, 1944, p. R-376.

Primary Examiner—Albert W. Davis, Jr.

Assistant Examiner—S. J. Richter

Attorney—James R. Hoatson, Jr. et al.

## [57] ABSTRACT

In the method of retarding corrosion of a heat exchanger being used to cool hot hydrocarbon vapors from a crude column by adding water to said vapors, the improvement to reduce loss of heat available in said exchanger by adding said water only for a time of from about 0.5 to about 2 hours within a 24 hour period.

6 Claims, No Drawings

## CRUDE OIL HEAT EXCHANGE

## BACKGROUND OF THE INVENTION

In the processing of crude oil, general practice is to first subject the crude oil to a desalting treatment. The desalted oil then is subjected to steam stripping in a crude column, with the vapors being taken overhead and the heavier products being withdrawn as side streams and bottoms product. The overhead vapors from the crude column are cooled and condensed by first being passed into indirect heat exchange with the crude oil charge and then by further cooling and condensing.

While much of the corrosive components of the crude oil are removed in the desalting operation, the crude oil still contains some metal chlorides (particularly calcium chloride and magnesium chloride) which decompose to release hydrogen chloride. In order to neutralize the acidic corrosives, it is general practice to introduce ammonia, morpholine or other basic reagent into the crude column overhead vapor line. Preferably a basic corrosion inhibitor, particularly of the film forming type, also is introduced into the vapor line. To still further reduce corrosion, it is general practice to continuously introduce water into the vapor line ahead of the heat exchanger, thereby to flush down ammonium chloride which is present in the overhead vapor line. One improvement in this method of operation is the reuse of the water collected in the receiver into which the condensed vapors pass.

## DESCRIPTION OF THE INVENTION

While the continuous introduction of water into the overhead vapor line serves to reduce corrosion in the heat exchanger and communicating equipment, this procedure has the disadvantage of reducing the amount of heat available in the exchanger. As hereinbefore set forth, the incoming crude oil charge is passed into indirect heat exchange with the hot vapors from the crude column. The heated crude oil charge then is supplied to conventional desalting operation. It is important that the temperature of the desalting be sufficiently high to accomplish efficient desalting of the crude oil. Accordingly, for economical purposes, it is desirable that the heat available in the heat exchanger be kept at a maximum so that such heat may be used to heat the incoming crude oil to a sufficiently high temperature for effective desalting treatment. Otherwise it may be necessary to utilize other means to obtain such heating and such other means entail additional equipment and cost.

The present invention is based on the principle that sufficient removal of acidic corrosives may be effected by only a part-time flushing with water. It is believed that corrosion in the heat exchanger and following equipment is caused by the deposition of solid ammonium chloride, which occurs upon cooling of the vaporous acidic corrosives. One theory is that ammonium chloride catalyzes sulfide corrosion, apparently through the reaction of the ammonium chloride with the sulfur containing compounds to form some ammonium sulfide compound or complex which, in turn, forms a first stage iron sulfide type corrosion and, if not removed, continues to corrode the metal. It is understood that the present applicant does not wish to be limited to this explanation but it does appear to be a reasonable explanation of the mechanism.

As hereinbefore set forth, upon cooling, ammonium chloride solidifies and, if allowed to remain, causes corrosion of the heat exchanger tubes. Generally, the overhead vapor fraction is withdrawn at a temperature of from about 250° to about 350° F. and is progressively cooled in the first exchanger to from about 200° to about 300° F. and in the second heat exchanger to from about 150° to 250° F. While additional heat exchangers may be used, in most cases one or more water cooled condensers are utilized to reduce the temperature of the vapors down to about ambient temperature. It is understood that these temperature ranges are typical only, and will vary with the specific procedure employed at a particular refinery.

As hereinbefore set forth, it is general practice to continuously flush the ammonium chloride down through the heat exchangers and condensers by introducing water at the inlet of the first heat exchanger. Accordingly, the water contacts the ammonium chloride before it is allowed to solidify. However, in accordance with the present invention it is believed that substantially the same objective is accomplished by introducing the water for only a comparatively short time instead of continuously as heretofore believed necessary. This is based upon the recognition that ammonium chloride undergoes very slow deposition and, by the periodical flushing herein proposed, will be washed out of the heat exchangers and condensers sufficiently to avoid corrosion of the steel equipment.

From the above discussion, it will be seen that the advantages of the water flushing of the acidic corrosives is retained without the disadvantages of reducing the heat available for use to heat the incoming crude oil charge. In other words, instead of the continuous loss in available heat, such loss is encountered for only a short period of time. This novel method offers an important economical advantage in the operation of the process.

The water to be introduced into the overhead vapor line may come from an outside source or conveniently is water collected in the receiver and reused for this purpose. As hereinbefore set forth, conventional practice is to pass the hot hydrocarbon vapors down through one or a plurality of heat exchangers, then through one or a plurality of water condensers and finally collected in a receiver. Because the crude column normally is subjected to water stripping, the overhead vapors contain the water which ultimately is collected in the receiver. Because this water does not contain undesirable impurities, as for example oxygen, reuse of this water for this purpose is particularly desirable. Accordingly, there is a large volume of such water available for such reuse.

The amount of water to be commingled with the crude column overhead vapors will be determined by the amount necessary to accomplish satisfactory removal of the acidic corrosives. As a practical matter, the amount of this water will be determined by the pumping and piping capacity available at the particular refinery. In any event, the introduction of the water will be limited for a time of from about 0.5 to about 2 hours and still more particularly from about 0.75 to about 1.5 hours within a 24 hour period. Excess water from the receiver is withdrawn from the system and, as another advantage to the process of the present invention, the withdrawal of the excess water also serves to remove

from the system the dissolved ammonium chloride and other acidic corrodents.

In view of the fact that the desalting and crude column operations are well known in the industry, there appears no need to describe such well-known procedures in detail in the present application. For example, R. H. Carlton U.S. Pat. No. 3,189,537 describes the continuous reuse of water collected in the receiver and the drawing illustrates a typical system. The drawing and description thereof in this patent, as well as the discussion of suitable film forming inhibitors and other details of operation, may be considered as the prior art and embodied in the present application as to details not repeated herein in the interest of brevity.

The following examples are introduced to illustrate further the novelty and utility of the present invention but not with the intention of unduly limiting the same.

#### EXAMPLE I

In this example, the crude column is connected to two heat exchangers and two condensers. Steam is introduced into the lower portion of the crude column at a rate of 2250 pounds per hour. The overhead vaporous fraction is withdrawn at a rate of 7500 barrels per day and at a temperature of 275° F. and a pressure of 9 p.s.i.g. Ammonia is introduced into the vapor line at a rate of 50 pounds per day and a corrosion inhibitor is introduced at a concentration of 20 parts per million based on the overhead vapor. The inhibitor is introduced downstream from the ammonia injection, but before the mixture is passed into the first heat exchanger. The inhibitor is a dibasic acid of a high molecular weight alkyl amine. In the first heat exchanger, the vaporized overhead is cooled to about 240° F. and further cooled in the second heat exchanger to a temperature of about 200° F. Crude oil being charged to the process is passed successively through the second heat exchanger and the first heat exchanger, after which it is further heated and then sent to the desalter. The overhead effluent, after passing through the second heat exchanger, is finally cooled in the condensers to a temperature of 90° F. and is collected at this temperature and a pressure of 5 p.s.i.g. in the receiver.

In accordance with the present invention, water separated in the receiver is commingled with the overhead vapors prior to solidification of ammonium chloride. The water is introduced into the vapor line ahead of the first exchanger. The reuse water is supplied at a rate of 30 gallons per minute for a period of 45 minutes during each 24 hours. Excess water containing dissolved ammonium chloride and other acidic corrodents is withdrawn from the receiver and utilized for any desired purpose or disposed of in any suitable manner.

#### EXAMPLE II

In this example the crude column is preceded by a

preflashing system. The preflash crude is supplied to the crude column which is maintained at a pressure of 14 p.s.i.g. Steam is introduced to the crude column at a rate of 1000 pounds per hour. A naphtha overhead is removed at a rate of 9400 barrels per day and a temperature of 310° F. Ammonia is introduced into the upper portion of the crude column at a rate of 70 pounds per day and a corrosion inhibitor is introduced at a concentration of 30 parts per million based upon the overhead vapor. The overhead vapor is withdrawn at a temperature of 310° F. and then is cooled in a heat exchanger in which the overhead vapor is passed in indirect heat exchange with the crude oil. In the heat exchanger, the overhead vapor is cooled to a temperature of 250° F. and then is further passed through two condensers and finally collected in the receiver at a temperature of 90° F. Prior to the use of the reuse water, corrosion was observed in the heat exchanger.

Water from the receiver is injected ahead of the heat exchanger at a rate of 40 gallons per minute for a time of 60 minutes in each 24 hour period. Excess water is removed from the receiver and utilized as desired or disposed of in any suitable manner.

The reuse water supplied in the manner described above serves to retard corrosion of the carbon steel heat exchanger tubes.

I claim as my invention:

1. In the method of retarding corrosion of a heat exchanger being used to cool hot ammonium chloride-containing hydrocarbon vapors from a crude column by adding water to said vapors, the improvement to reduce loss of heat available in said exchanger, which comprises adding said water prior to solidification of the ammonium chloride and only for a time of from about 0.5 to about 2 hours within a 24 hour period.
2. The method of claim 1 in which incoming crude oil is passed into indirect heat exchange with said hydrocarbon vapors.
3. The method of claim 1 in which said water is added only for a time of from about 0.75 to about 1.5 hours within a 24 hour period.
4. The method of claim 1 in which said water is at least a part of the water collected in the receiver into which the cooled hydrocarbon vapors pass.
5. The method of claim 1 in which said water is added to the hydrocarbon vapors prior to entering the heat exchanger.
6. The method of claim 5 wherein a plurality of heat exchangers and condensers are used in the cooling and condensing of said hot hydrocarbon vapors, and the water is injected ahead of the first heat exchanger.

\* \* \* \* \*